# EUROPEAN PATENT SPECIFICATION

(11) **EP 2 001 822 B1**
(45) Date of publication and mention of the grant of the patent: **16.08.2017**
(21) Application number: 07727712.7
(22) Date of filing: 03.04.2007
(51) Int. Cl.: C06B 45/00, C06D 5/06, C06B 21/00

(54) **PYROTECHNIC GRAINS OF LARGE DIMENSIONS, AND THEIR PRODUCTION AND USE**
PYROTECHNISCHE KÖRNER MIT GROSSEN ABMESSUNGEN UND IHRE HERSTELLUNG UND VERWENDUNG
GRANULES PYROTECHNIQUES DE GRANDES DIMENSIONS, LEUR PRODUCTION ET LEUR UTILISATION

(30) Priority: 04.04.2006 FR 0651183
(43) Date of publication of application: 17.12.2008
(73) Proprietor: HERAKLES, 33185 Le Haillan (FR)
(72) Inventor: BLANCHARD, Hélène, F-92340 Bourg La Reine (FR); BODART, Vincent, F-75014 Paris (FR); ROCTON, Hugues, F-91710 Vert Le Petit (FR)
(74) Representative: Le Roux, Martine
(86) International application number: PCT/EP2007/053241
(87) International publication number: WO 2007/113299

(56) References cited:
- WO-A-95/00205
- WO-A-2004/024653
- WO-A2-2006/134311
- FR-A1- 2 864 905
- FR-A1- 2 870 459
- US-A- 4 998 751
- US-A- 5 682 013
- US-A1- 3 814 694
- US-A1- 5 500 059
- US-A1- 5 641 938
- US-A1- 2004 173 922
- US-A1- 2004 216 819

## Description

The present invention relates to large pyrotechnic grains based on binder-free formulations, to their production, and to their use. More precisely, it relates to:
- pyrotechnic grains which are in the form of blocks (monolithic blocks) with large dimensions;
- a method of producing them; and
- a method of generating gas comprising the combustion of said grains.

Gas generation has a number of applications, both in the civilian and in military fields.

In the automotive safety sector, gas generators have been developed with a short operational duration, which use compositions with a high combustion rate. Those compositions are in the form of thin pellets (1 mm [millimeter] to 3 mm) with a small diameter (3 mm to 7 mm). This provides them with a large combustion surface, encouraging a high rate over a short period (necessary for airbag applications in automotive safety, of the driver's airbag type). The porosity of such pellets is generally less than 4%. Pelletization operations carried out to produce said pellets are well known, similar to those used in medicinal formulations. Compositions based on guanidine nitrate and basic copper nitrate have been used in that context (United States patent US-A_5 608 183 and United States Patent Application Publication 2004/0173922 A1). An attempt has even been made to improve the combustion rate (US-A-6 143 102) since said combustion rate of such compositions is rather low, compared with that of other compositions used in the same field.

In similar sectors (automotive safety, to inflate curtain types of airbag which need to remain inflated for a long period), or in completely different sectors, gas generators have been proposed, especially for:
- inflating or deforming a structure;
- propelling a liquid or a gas;
- actuating a jack or some other mechanical actuator;
- causing a displacement.

Generating and supplying gas has also been exploited to operate fire extinguishing devices (FR-A-2 864 905 and FR-A-2 870 459).

That relates to the field of slow gas generation. For slowly generating and supplying gas under pressure, a gas stored under pressure is generally used. The use of chemical reactions or the combustion of pyrotechnic cartridges has also been mentioned. With the combustion of pyrotechnic cartridges, the flow rate of the gas that is generated is controlled by selecting the characteristics of the propellant, the geometry of the cartridges, and/or the conditions for ejecting said generated gas, etc.

The present invention falls within the context of generators operation providing long duration, low flow rate, and low operating pressure.

In such a context, the present invention proposes pyrotechnic grains that are simple in shape and that satisfy the following specifications:
a) a long combustion period (50 ms [millisecond] to 1 min [minute]) due to a slow combustion rate (to ensure a long period of operation) and/or to a ratio of combustion area over burning thickness that is low, and/or to a low operating pressure (for use in low pressure generators and to encourage a low combustion rate);
b) low dependency of the rate of combustion on the operating temperature of the grain, to ensure good ballistic behavior under extreme temperature conditions from -60°C to 110°C (hence an extension of the application range (see below), especially in aeronautics);
c) suitable mechanical behavior (without the intervention of a binder, the presence of which would deleteriously affect ballistic performance), especially encouraging the use of said grains in an aggressive vibratory environment.

The pyrotechnic grains of the invention are also advantageously non-aggressive for the gas generator in which they are used and for the associated system (i.e., on combustion, they generate neither particles nor corrosive species). In the same manner, the generated species are advantageously of low toxicity.

Referring to point a) of the above specifications, the skilled person will understand that the pyrotechnic grain of the invention must be thick and have a small combustion area. Thus, it must be a large grain, larger than the pellets mentioned above.

Referring to point b) of the above specifications, the skilled person will know that said grain must have low porosity.

Said skilled person will also be aware of the difficulties in fabricating a large grain of that type (pyrotechnic grain) with low porosity, with appropriate mechanical behavior, and without using a binder. He knows that pyrotechnic grains of large dimensions and without binder in their composition have generally porosity values which are not acceptable in reference to their ballistic properties, more particularly their combustion rate. This point is all the more crucial than their operating temperature is high.

Surprisingly, the Applicant has obtained pyrotechnic grains, from specific oxidizing and reducing charges, which are simple in shape and that satisfy the above specifications. Such pyrotechnic grains constitute the first aspect of the present invention.

Said pyrotechnic grains of the invention have a composition that comprises at least one (specific) oxidizing charge and at least one (specific) reducing charge, but that includes no binder. In this respect, they are pyrotechnic grains of the pellet type mentioned above. The composition of the pyrotechnic grains of the invention generally essentially consists of at least one such (specific) oxidizing charge and at least one such (specific) reducing charge. It generally essentially consists of a (specific) oxidizing charge (an oxidizer) and a (specific) reducing charge (a reducer).

Said at least one specific oxidizing charge comprises basic copper nitrate. Preferably it consists of basic copper nitrate.

Said at least one specific reducing charge comprises guanidine nitrate. Preferably it consists of guanidine nitrate.

In characteristic manner, said pyrotechnic grains of the invention have a composition which comprises:
- 45% to 55% by weight of guanidine nitrate;
- 40% to 50% by weight of basic copper nitrate;
- 0 to 5% by weight of additives ; and
no binder; and
are in the form of substantially cylindrical blocks:
- with a thickness of 7.5 mm or more;
- with an equivalent diameter of 20 mm or more; and
- with porosity in the range 1% to 8%, limits included.

Said (monolithic) blocks are large blocks, which are simple in shape and of low porosity.

Said blocks have a substantially cylindrical shape. Generally, but not exclusively, they are circular cylinders or near (quasi) circular cylinders.

The shape of the grains of the invention is the signature of the last step of the method by which they are obtained: a compacting step (see below).

Said blocks may in particular consist of solid (quasi) cylinders or (quasi) cylindrical sleeves.

The grains in question are large objects (thickness of at least 7.5 mm, equivalent diameter (or, clearly, diameter if it is a perfect circular cylinder) of 20 mm or more), and are relatively dense (porosity in the range 1% to 8%).

Non-limiting dimensions of said grains are detailed below. Generally and independently :
- the thickness of the blocks is 75 mm or less; or
- the equivalent diameter of said blocks is 75 mm or less.

In general, said thickness and said equivalent diameter are both 75 mm or less.

According to an advantageous embodiment:
- the thickness of the blocks is in the range 10 mm to 60 mm (values of 10 mm and 60 mm being included).

In particular, pyrotechnic blocks of the solid circular cylinder type and with the dimensions given below, have been produced in the context of the invention:
- diameter of 25 mm and thickness of 10 mm;
- diameter of 50 mm and thickness of 50 mm.

Further, it has been stated that the porosity of the blocks is in the range 1% to 8% (it should be noted here that this parameter, expressed as a percentage, corresponds to the ratio between the actual density and the theoretical density; it is in fact the difference from the theoretical density).

Said porosity is advantageously 5% or less. It should be recalled that the lower said porosity, the lower the dependency of the rate of combustion on the operating temperature of the grain.

It should be indicated here that, in a non-limiting manner, blocks, which are of the circular cylinder type with the dimensions described above, have been respectively obtained with the porosities indicated below :
- porosity of about 5% (with diameter = 25 mm and thickness = 10 mm);
- porosity of about 7% (with diameter = thickness = 50 mm).

As indicated above, the pyrotechnic grains of the invention, which are simple in shape, being substantially cylindrical, may in particular consist of solid cylinders or sleeves. The equivalent internal diameter of said sleeves is advantageously more than 10 mm; preferably, it is in the range 12 mm to 35 mm (that implies obviously a greater equivalent diameter of the sleeve).

Referring to the composition of the pyrotechnic grains of the invention, the following non-limiting details can furthermore be given.

The said composition of the pyrotechnic grains of the invention includes basic copper nitrate as the oxidizing charge and guanidine nitrate as the reducing charge. Advantageously, it comprises basic copper nitrate as the only oxidizing charge and guanidine nitrate as the only reducing charge. In the automotive safety field (driver type airbags), said basic copper nitrate/guanidine nitrate combination is known to have a combustion rate that is rather low relative to that of other compositions used in this field. In the context of this advantageous embodiment, said composition also comprises:
- 45% to 55% by weight of guanidine nitrate;
- 40% to 50% by weight of basic copper nitrate; and
- 0 to 5% by weight of additives.

The additives in question, which are optionally present, are chemical compounds that are known per se as well as for their beneficial involvement in the general production of pyrotechnic grains. In particular, they may be:
- slagging agents supplied with the starting materials : oxidizing charge(s) and reducing charge(s) (for example: alumina);
- processing aids of the pressing aid or unmolding aid type (for example: silica, calcium stearate, mica, etc).

In a second aspect, the present invention provides the production of large pyrotechnic grains, as described above.

The method in question comprises a series of steps that are known *per se.*

Surprisingly, it has been possible to find operating conditions for this series of steps (which are known *per se*) that enable, from the selected oxidizing and reducing charges, grains of the invention to be obtained without the involvement of a binder, and having simultaneously large dimensions, low porosity, and also acceptable mechanical properties (which can tolerate the vibrational environment of an automobile or aircraft).

The method of producing pyrotechnic grains of the invention comprises carrying out the following steps in succession:
- intimately dry or wet mixing said oxidizing (basic copper nitrate) and reducing (guanidine nitrate) charges used in the powder state and in suitable relative amounts;
- dry or wet granulating the powdered mixture obtained;
- sizing the granules obtained; and
- shaping the retained sized granules by compacting ;
under conditions that produce the anticipated result, i.e. the production of pyrotechnic grains having the dimensional and porosity characteristics defined above.

The conditions in question are principally:
- the characteristics of the starting powders ;
- the characteristics of the retained sized granules; and
- the compacting parameters.

The Applicant has discovered that suitable conditions may be combined to obtain the desired result.

Before detailing said conditions (parameters) of the method of the invention, it should in general be indicated:
- that the powders are advantageously intimately dry mixed ;
- that granulation is also advantageously a dry granulation (independently of the manner of said intimate mixing) ;
- that the granules are advantageously sized by sieving; and
- that at least one shaping additive (a pressing aid, such as calcium stearate or mica) may advantageously be added to said sized granules before shaping them by compacting.

In characteristic manner, to obtain the anticipated result, more particularly to obtain a slow rate of combustion, at least one of the charges used in the powder state has a median diameter that is substantially larger than that which is used in the prior art to prepare pellets (of small dimensions). Thus, it is recommended in the context of carrying out the method of the present invention to use at least part of the reducing charge(s) with a median diameter that is substantially higher (× 4, × 6) than that known to be used in the preparation of prior art pellets. It is recommended that guanidine nitrate with a median diameter of 200 µm [micrometer] or more be used. In particular, it is recommended that guanidine nitrate with a median diameter of 200 µm to 300 µm be used. Said guanidine nitrate is conventionally used for the fabrication of pellets, with a median diameter of 50 µm.

In characteristic manner, to obtain the anticipated result, more particularly to obtain low porosity, the granules selected are those that have a median diameter of more than 200 µm, preferably in the range 500 µm to 1000 µm. It is thus recommended, in the context of the present invention, that basic copper nitrate/guanidine nitrate granules with a median diameter in the range 500 µm to 700 µm be selected.

The skilled person is capable of optimizing this parameter (granule size) as well as the others (powder mean diameter and compacting parameters) as a function of the exact nature of the products in question.

Regarding the compacting parameters, in general, to obtain the anticipated result, more particular to obtain low porosity, a pressure in the range 15 × 10⁶ Pa [pascal] to 35 × 10⁶ Pa is applied for 0.1 s [second] to 30 s.

Compacting is clearly carried out in a mold the shape of which corresponds to that envisaged for the prepared pyrotechnic grain (substantially cylindrical shape).

The method of the invention is very advantageously carried out with all the above advantageous embodiments, i.e.:
- a median diameter of guanidine nitrate of 200 µm or more ;
- a median diameter of the granules of more than 200 µm ; and
- a compacting step carried out at 15-35 x 10⁶ Pa during 0.1 to 30 s.

The method of the invention is advantageously carried out with a basic copper nitrate/guanidine nitrate combination. In the context of the present invention, the combustion rate of compositions based on these two elements (BCN/GN) is reduced. The teaching of the present invention thus goes against that of US-A-6143 102.

In a third aspect, the present invention provides a method of generating gas, the method comprising, in conventional manner, the combustion of at least one pyrotechnic grain. In characteristic manner, said method of the invention comprises the combustion of at least one pyrotechnic grain as described above (large pyrotechnic grain) and/or produced using the method described above.

Said gas generation method is carried out in a suitable device which, in particular, has a combustion chamber adapted to the dimensions of the original pyrotechnic charge, based on large pyrotechnic grains. In common with currently known devices, said device comprises:
- elements for retaining, positioning, and adjusting the pyrotechnic charge based on large pyrotechnic grains (which constitutes the first aspect of the present invention);
- ignition elements;
- at least one safety cap ensuring depressurization of the generator in the event of accidental overpressure;
- at least one nozzle; and
- a filter to retain the majority of the solid combustion residues.

Interesting applications for the pyrotechnic grains of the invention are specified below, i.e. fields in which gas generation must be maintained for a relatively long period.

The following applications are particularly contemplated:
- the generation of gas intended to propel a fluid, either directly or via a separating membrane, for example, to extinguish fire in civilian or military aircraft engines, to inert bays in civilian or military aircraft, to extinguish fire in a building, in all types of civilian vehicles (automobiles, etc) or military vehicles (tanks, etc), to inject grease or active principle, etc;
- the generation of gas in a pyrotechnic actuator intended to actuate a jack, for example (to open an aircraft door, for example);
- the generation of gas to inflate or deform inflatable structures that are deformable, such as aircraft escape chutes, automotive safety anti-submarining structures, or releasers.

Finally, examples of the present invention are described below.

### Example 1

Pyrotechnic grains of the invention were prepared from the following starting materials:
- basic copper nitrate (BCN): powder with a median diameter of 8 µm;
- guanidine nitrate (GN): powder with a median diameter of 218 µm;
- alumina (slagging agent): powder with a median diameter of 1 µm.

Said powders were dry mixed in a Sofraden^{®} type powder mixer (a Guédu^{®} type mixer would also have been suitable) in the following proportions:

| | |
|---|---|
| BCN | 44.87% |
| GN | 52.44% |
| Alumina | 2.69% (weight %). |

The intimate mixture of powders obtained was dry granulated in a Sahut Conreur^{®} type granulator (an Alexanderwerk^{®} type granulator would also have been suitable). Said intimate mixture of powders was forced through a screen. The granulometric distribution of the granules obtained was from 10 µm to 1000 µm.

The granules obtained were then sieved, and those with a mean diameter of more than 200 µm were selected.

Said selected granules were then compacted on a 35 (metric) tonne single action press. The compacting pressure applied was 230 bars (23 × 10⁶ Pa). It was applied for 10 s.

Pyrotechnic grains in accordance with the invention were obtained, which grains were cylindrical monoliths (shape of mold) with a thickness of 10 mm, a diameter of 24.6 mm, and porosity of 3%.

### Example 2

In similar manner, cylindrical grains were prepared as follows:
- with a thickness of 50 mm;
- with a diameter of 50 mm;
- with porosity of 7%.

### Example 3 (prior art)

In similar manner, prior art pellets, which were cylindrical grains, were prepared as follows:
- with a thickness of 1.8 mm;
- with a diameter of 6.3 mm;
- with porosity of 2%.

The grains of said Examples 1 to 3 were tested in generators with the same architecture. The graphs of the operating pressures of said generators as a function of time are given in the accompanying Figures 1 to 3.

With the prior art pellet, as expected, an operating peak was obtained (Figure 3). With the blocks of the invention, the desired spread over time was observed (Figures 1 and 2).

Further, the mechanical behavior of the grains of the invention as regards aeronautical vibrations was tested, with satisfactory results (standard RTCA DO-160D: "Environmental Conditions and Test Procedures for Airborne Equipment").

## Claims

1. A pyrotechnic grain,
the composition of which comprises:
· 45% to 55% by weight of guanidine nitrate;
· 40% to 50% by weight of basic copper nitrate;
· 0 to 5% by weight of additives; and
no binder;
in the form of a substantially cylindrical block:
· with a thickness of 7.5 mm or more;
· with an equivalent diameter of 20 mm or more; and
· with porosity in the range 1% to 8%, limits included.

2. The pyrotechnic grain according to claim 1, **characterized in that** the thickness of said block is in the range 10 mm to 60 mm, limits included.

3. The pyrotechnic grain according to claim 1 or 2, **characterized in that** the porosity of said block is 5% or less.

4. The pyrotechnic grain according to any one of claims 1 to 3, **characterized in that** it is in the form of a sleeve of internal equivalent diameter that is advantageously more than 10 mm.

5. The pyrotechnic grain according to any one of claims 1 to 4, **characterized in that** basic copper nitrate is the only oxidizing charge.

6. The pyrotechnic grain according to any one of claims 1 to 5, **characterized in that** guanidine nitrate is the only reducing charge..

7. A method of producing a pyrotechnic grain according to any one of the preceding claims, **characterized in that** it comprises:
· intimately dry or wet mixing guanidine nitrate and basic copper nitrate used in the powder state and in suitable relative amounts;
· dry or wet granulating the powdered mixture obtained;
· sizing the granules obtained; and
· shaping the retained sized granules by compacting;
the characteristics of the starting powders, the retained sized granules and the compacting parameters being selected to produce said pyrotechnic grains having said dimensional and porosity characteristics.

8. The method according to claim 7, **characterized in that** the intimate mixture or (and) granulation is (are) carried out by a dry method.

9. The method according to claim 7 or 8, **characterized in that** the granules are sized by sieving.

10. The method according to any one of claims 7 to 9, **characterized in that** it comprises:
· using guanidine nitrate with a median diameter of 200 µm or more; and/or, advantageously and
· sieving the granules to retain those with a median diameter of more than 200 µm; and/or, advantageously and
· shaping by compacting at a pressure in the range 15 × 10⁶ Pa to 35 × 10⁶ Pa for 0.1 s to 30 s.

11. The method according to any one of claims 7 to 10, **characterized in that** it is carried out with guanidine nitrate as the only reducing charge and basic copper nitrate as the only oxidizing charge.

12. A method of generating gas, comprising the combustion of at least one pyrotechnic grain, **characterized in that** said at least one pyrotechnic grain is a grain according to any one of claims 1 to 6 and/or a grain produced according to any one of claims 7 to 11.

## Patentansprüche

1. Pyrotechnisches Gegenstand,
dessen Zusammensetzung umfasst:
45 bis 55 Gewichts-% Guanidinnitrat,
40 bis 50 Gewichts-% basisches Kupfernitrat,
0 bis 5 Gewichts-% Hilfsstoffe und
kein Bindemittel,
in Form eines im Wesentlichen zylindrischen Blocks
mit einer Dicke von 7,5 mm oder mehr,
mit einem äquivalenten Durchmesser von 20 mm oder mehr und
mit einer Porosität im Bereich von 1 bis 8 %, Grenzen eingeschlossen.

2. Pyrotechnisches Gegenstand nach Anspruch 1, **dadurch gekennzeichnet, dass** die Dicke des Blocks im Bereich von 10 bis 60 mm liegt, Grenzen eingeschlossen.

3. Pyrotechnisches Gegenstand nach Anspruch 1 oder 2, **dadurch gekennzeichnet, dass** die Porosität des Blocks 5 % oder weniger beträgt.

4. Pyrotechnisches Gegenstand nach einem der Ansprüche 1 bis 3, **dadurch gekennzeichnet, dass** es in Form einer Hülse mit einem internen äquivalenten Durchmesser vorliegt, der vorteilhafterweise mehr als 10 mm beträgt.

5. Pyrotechnisches Gegenstand nach einem der Ansprüche 1 bis 4, **dadurch gekennzeichnet, dass** das basische Kupfernitrat die einzige oxidierende Ladung ist.

6. Pyrotechnisches Gegenstand nach einem der Ansprüche 1 bis 5, **dadurch gekennzeichnet, dass** das Guanidinnitrat die einzige reduzierende Ladung ist.

7. Verfahren zum Herstellen eines pyrotechnischen Gegenstands nach einem der vorhergehenden Ansprüche, **dadurch gekennzeichnet, dass** es umfasst:
inniges Trocken- oder Nassmischen von Guanidinnitrat und basischem Kupfernitrat, die in Pulverform und in geeigneten relativen Mengen verwendet werden,
Trocken- oder Nassgranulieren der erhaltenen pulverisierten Mischung,
Größeneinteilung der erhaltenen Granula und
Formen der zurückbehaltenen größeneingeteilten Granula mittels Verdichten,
wobei die Eigenschaften der Anfangspulver, der zurückbehaltenen größeneingeteilten Granula und der Verdichtungsparameter ausgewählt sind, um das pyrotechnische Gegenstand herzustellen, das die besagten Dimensions- und Porositätseigenschaften aufweist.

8. Verfahren nach Anspruch 7, **dadurch gekennzeichnet, dass** die innige Mischung und/oder Granulierung mittels eines Trockenverfahrens ausgeführt wird/werden.

9. Verfahren nach Anspruch 7 oder 8, **dadurch gekennzeichnet, dass** die Granula mittels Sieben größeneingeteilt werden.

10. Verfahren nach einem der Ansprüche 7 bis 9, **dadurch gekennzeichnet, dass** es umfasst:
Verwenden von Guanidinnitrat mit einem mittleren Durchmesser von 200 µm oder mehr und/oder, vorteilhafterweise und,
Sieben der Granula, um solche mit einem mittleren Durchmesser von mehr als 200 µm zurückzubehalten, und/oder, vorteilhafterweise und,
Formen mittels Verdichten bei einem Druck im Bereich von 15 x 10⁶ Pa bis 35 x 10⁶ Pa für 0,1 bis 30 s.

11. Verfahren nach einem der Ansprüche 7 bis 9, **dadurch gekennzeichnet, dass** es mit Guanidinnitrat als der einzigen reduzierenden Ladung und mit basischem Kupfernitrat als der einzigen oxidierenden Ladung ausgeführt wird.

12. Verfahren zum Erzeugen eines Gases, umfassend Verbrennen wenigstens eines pyrotechnischen Gegenstands, **dadurch gekennzeichnet, dass** das wenigstens eine pyrotechnische Gegenstand ein Gegenstand nach einem der Ansprüche 1 bis 6 und oder ein nach einem der Ansprüche 7 bis 11 hergestelltes Gegenstand ist.

## Revendications

1. Objet pyrotechnique
dont la composition comprend :
▪ 45 % à 55 % en masse de nitrate de guanidine ;
▪ 40 % à 50 % en masse de nitrate basique de cuivre ;
▪ 0 à 5 % en masse d'additifs ; et
pas de liant ;
sous la forme d'un bloc sensiblement cylindrique :
▪ dont l'épaisseur est de 7,5 mm ou plus;
▪ dont le diamètre équivalent est de 20 mm ou plus; et
▪ dont la porosité est comprise entre 1 % et 8 %, valeurs limites incluses.

2. Objet pyrotechnique selon la revendication 1, **caractérisé en ce que** l'épaisseur dudit bloc est comprise entre 10 mm et 60 mm, valeurs limites incluses.

3. Objet pyrotechnique selon la revendication 1 ou 2, **caractérisé en ce que** la porosité dudit bloc est de 5 % ou moins.

4. Objet pyrotechnique selon l'une quelconque des revendications 1 à 3, **caractérisé en ce qu'**il se présente sous la forme d'un manchon, dont le diamètre équivalent interne est avantageusement de plus de 10 mm.

5. Objet pyrotechnique selon l'une quelconque des revendications 1 à 4, **caractérisé en ce que** le nitrate basique de cuivre est l'unique charge oxydante.

6. Objet pyrotechnique selon l'une quelconque des revendications 1 à 5, **caractérisé en ce que** le nitrate de guanidine est l'unique charge réductrice.

7. Procédé d'obtention d'un objet pyrotechnique selon l'une quelconque des revendications précédentes, **caractérisé en ce qu'**il comprend :
- le mélange intime, mis en oeuvre par voie sèche ou par voie humide, du nitrate de guanidine et du nitrate basique de cuivre utilisés à l'état de poudre et en quantité relatives adéquates ;
- la granulation, mise en oeuvre par voie sèche ou par voie humide, du mélange pulvérulent obtenu ;
- le calibrage des granulés obtenus ; et
- la mise en forme des granulés calibrés retenus par compactage ;
les caractéristiques des poudres de départ, des granulés calibrés retenus ainsi que les paramètres du compactage étant choisis pour l'obtention dudit objet pyrotechnique aux caractéristiques, de dimensionnement et de porosité, énoncées.

8. Procédé selon la revendication 7, **caractérisé en ce que** le mélange intime ou(et) la granulation est(sont) mis en oeuvre par voie sèche.

9. Procédé selon la revendication 7 ou 8, **caractérisé en ce que** les granulés sont calibrés par tamisage.

10. Procédé selon l'une quelconque des revendications 7 à 9, **caractérisé en ce qu'**il comprend :
. l'emploi de nitrate de guanidine dont le diamètre médian est de 200 µm ou plus ; et/ou, avantageusement et
. le tamisage des granulés pour retenir ceux dont le diamètre médian est de plus de 200 µm ; et/ou, avantageusement et
. la mise en forme par compactage à une pression comprise entre 15 x 10⁶ Pa et 35 x 10⁶ Pa pendant 0,1 s à 30 s.

11. Procédé selon l'une quelconque des revendications 7 à 10, **caractérisé en ce qu'**il est mis en oeuvre avec du nitrate de guanidine comme unique charge réductrice et du nitrate basique de cuivre comme unique charge oxydante.

12. Procédé de génération de gaz, comprenant la combustion d'au moins un objet pyrotechnique, **caractérisé en ce que** ledit au moins un objet pyrotechnique est un objet selon l'une quelconque des revendications 1 à 6 et/ou un objet obtenu selon l'une quelconque des revendications 7 à 11.
